

## UNITED STATES PATENT OFFICE.

FRANK F. COLCORD, OF NEW YORK, N. Y., ASSIGNOR TO UNITED STATES SMELTING, REFINING & MINING COMPANY, OF PORTLAND, MAINE, A CORPORATION OF MAINE.

## TREATMENT OF ANTIMONIAL METALS.

No Drawing.

Application filed November 22, 1923. Serial No. 676,354.

*To all whom it may concern:*

Be it known that I, FRANK F. COLCORD, a citizen of the United States, residing at New York city, in the county of New York and State of New York, have invented certain new and useful Improvements in the Treatment of Antimonial Metals; and I do hereby declare the following to be a full, clear, and exact description of the invention, such as will enable others skilled in the art to which it appertains to make and use the same.

The invention relates to the treatment of antimonial metals or alloys for the removal of such impurities as arsenic or arsenic and copper.

I have found that arsenic present in antimonial metals or alloys such as antimonial lead may be conveniently and economically removed without appreciable effect upon the antimony by treating the molten alloy with caustic alkali, such as caustic soda, or an alkali salt, such as soda ash, at suitable temperatures above those at which the salts or caustic melt.

The invention is of particular value as applied to the purifying of antimonial lead alloys whether produced by the mixing of metals or as a product in metallurgical refining operations and will be further explained in connection with the purifying of antimonial lead alloy such as usually produced in the refining of lead bullion. Such alloys usually contain small percentages of arsenic and copper say from  $\frac{1}{10}$  to  $1\frac{1}{2}\%$  arsenic and from  $\frac{3}{10}$  to  $\frac{1}{5}\%$  copper. While for some uses the presence of these impurities is not particularly detrimental, it renders the alloys unfit for other fields of use.

In treating these alloys the preferred mode of operation is as follows: The molten alloy is brought to a temperature between 900° and 1000° F. and the caustic soda is added in about the proportion of three pounds of caustic to each pound of arsenic in the alloy. The total amount of caustic is best added in successive fractional additions, the number of such additions depending upon the amount of arsenic present and the degree to which it is to be removed. The caustic soda is thoroughly stirred into the molten alloy either mechanically or by blowing with air or steam. The stirring or agitation of the molten metal continues until the caustic is spent, which usually oc-

curs in about an hour. The skim thus formed is removed and then the treatment with caustic soda is repeated until by test the removal of the arsenic to the desired degree is shown. During the successive treatments with caustic soda the temperature of the molten metal is preferably maintained within an approximate range of from 900° to 1000° F. although somewhat lower and higher temperatures are permissible.

I have found that with the above method the arsenic may be economically and efficiently removed entirely or to any desired degree from antimonial lead alloys without materially affecting the antimony which is usually present in amounts from 4 to 20%. This method is also applicable to the purifying of antimony-tin-lead alloys as the caustic soda treatment will remove the arsenic from the molten alloy without affecting either the antimony or tin contained in an antimonial lead alloy of this character. It is also applicable to the purifying of such other antimonial metals or alloys as are of a character to admit of similar treatment at temperatures which will result in the removal of the arsenic without material effect on the antimony therein.

Similar results may be secured by like treatment with alkali salts such as soda ash although the range of temperature at which the treatment should be effected in order to secure the best results is somewhat higher than with caustic soda.

In case the alloy to be purified also contains copper as an impurity this may be removed either before or after, preferably before removal of the arsenic by treating the molten alloy with sulphur at a comparatively low temperature. The amount of sulphur to be added will vary with the amount of copper present and will be approximately one pound of sulphur to each pound of copper. The sulphur preferably, but not necessarily, in the form of flowers of sulphur, is thoroughly stirred into the molten alloy while the temperature is preferably maintained somewhat below the burning point of sulphur or at an approximate range of from 560° to 600° F. The copper will quickly unite with the sulphur and will float on the molten alloy in the form of dross. After the stirring has con-

tinued say for about half an hour it is stopped and the temperature of the molten metal lowered to about 550° F. and the dross containing the copper is then removed.

By the method described arsenic or arsenic and copper may be quickly and economically removed from antimonial lead alloys and other metals or alloys containing 10 antimony which are of a character to admit of treatment by this method and these alloys may thus be rendered fit for uses which require an alloy free from such impurities.

This application, so far as its subject 15 matter is disclosed in applicant's pending application, Serial No. 579,035, filed August 1, 1922, is a continuation of said application.

What is claimed is:

20 1. The method of purifying antimonial lead alloys which consists in subjecting the molten alloy to the action of an alkali at temperatures to cause the arsenic in the alloy to unite with the alkali without affecting the antimony.

25 2. The method of purifying antimonial lead alloys which consists in treating the molten alloy with caustic soda at a temperature above that at which the caustic 30 soda melts to remove the arsenic which is in the alloy without affecting the antimony.

35 3. The method of purifying antimonial lead alloys which consists in treating the molten alloy with caustic soda at an approximate temperature range of from 900° to 1000° F. to remove the arsenic which is in the alloy.

40 4. The method of purifying antimonial lead alloys which consists in treating the molten alloy with sulphur to remove the copper therefrom and with an alkali to remove the arsenic without affecting the antimony.

45 5. The method of purifying antimonial lead alloys which consists in treating the molten alloy with caustic soda at an approximate temperature range of from 900° to 1000° F. to remove the arsenic and with sulphur at an approximate temperature 50 range of from 550° to 600° F. to remove the copper.

55 6. The method of purifying antimonial lead alloys which consists in subjecting the molten alloy to agitation and simultaneously to the action of an alkali at temperatures to cause the arsenic in the alloy to unite with the alkali without affecting the antimony.

60 7. The method of purifying antimonial lead alloys which consists in agitating the

molten alloy and simultaneously treating it with caustic soda at an approximate temperature range of from 900° to 1000° F. to remove the arsenic which is in the alloy.

8. The method of purifying antimonial 65 metals which consists in subjecting the molten metal to the action of an alkali at temperatures to cause the arsenic in the metal to unite with the alkali without affecting the antimony.

9. The method of purifying antimonial 70 metals which consists in subjecting the molten metal to agitation and simultaneously to the action of an alkali at temperatures to cause the arsenic in the metal 75 to unite with the alkali without affecting the antimony.

10. The method of purifying antimonial 80 metals which consists in treating the molten metal with caustic soda at an approximate 85 temperature range of from 900° to 1000° F. to remove the arsenic which is in the metal.

11. The method of purifying antimonial 90 metals which consists in agitating the molten metal and simultaneously treating it with caustic soda at an approximate temperature range of 900° to 1000° F. to remove the arsenic which is in the metal.

12. The method of purifying antimonial 95 metals which consists in subjecting the molten metal to repeated treatment with an alkali at temperatures to cause arsenic in the metal to unite with the alkali without affecting the antimony.

13. The method of purifying antimonial 100 metals which consists in subjecting the molten metal to repeated treatments with caustic soda at an approximate temperature range of from 900° to 1000° F. to effect 100 fractional removal of the arsenic which is in the metal.

14. The method of purifying antimonial 105 metals which consists in intermingling caustic soda with the molten metal at an approximate temperature range of from 900° to 1000° F. to remove a part of the arsenic which is in the metal and repeating the treatment until the desired reduction in the arsenic is effected.

15. The method of purifying antimonial 110 metals which consists in subjecting the molten metal to the action of a caustic alkali at temperatures to cause the arsenic in the metal to unite with the alkali without affecting the antimony, and agitating the mixture during the treatment by blowing air therein.

FRANK F. COLCORD,